

## UNITED STATES PATENT OFFICE.

HAROLD G. WEIDENTHAL, OF CLEVELAND, OHIO, ASSIGNOR TO THE JAMES H. HERON COMPANY, OF CLEVELAND, OHIO, A CORPORATION OF OHIO.

## ALLOY.

No Drawing.

Application filed April 3, 1919. Serial No. 287,284.

This invention relates to alloys and has for its object the provision of an improved metallic composition, devised primarily for the purpose of making die-blocks and like tools for the working of hot metals, but of great value for many other purposes such as light armor, armor plate, gun liners, frogs and crossings of railways, dipper teeth, gas-engine valves and in many other 10 places where a hard and durable alloy is required which will stand either high temperature or severe mechanical wear. Further objects of the invention are the provision of a composition of this nature which shall be 15 made of comparatively inexpensive materials, shall be either oil hardening or air hardening and shall be little if any injured by overheating. It is also an object of the invention to produce a metal which can be readily forged, and easily welded, and conveniently machined when annealed or softened.

My improved alloy is most conveniently made by adding to steel of the proper carbon-content a predetermined amount of silicon together with the proper amount of chromium, preferably accompanied by a small amount of some scavenging agent such as uranium, vanadium, molybdenum, zirconium, or titanium. A specimen composition 20 which I have found to give extremely satisfactory results is as follows:

Chromium, 3% to 6%, silicon 1% to 2½%, carbon .30% to 1.00%, uranium (or equivalent) .10% to .30%, phosphorous, sulphur, 25 manganese as in normal steel specifications, iron by difference to make 100%.

The effect of the silicon is to afford a very high coefficient of elasticity, combined with great density, but normally accompanied by a rather abrupt elastic limit, at least for dynamic force. The effect of the chromium is to render the alloy air hardening when used in conjunction with the silicon. The hardness of the alloy will depend 40 to a very great extent upon the carbon content, running from quite soft (where annealed) at .30 carbon up to a super-hardness at 1.00 carbon (the usual practical limit being about .60%).

50 I have found uranium to produce a more satisfactory action in this alloy than any of the other substitutes therefor which I have named, yet any of the equivalents mentioned serve in my opinion to produce an alloy which is better than anything heretofore

known. I do not restrict myself to the quantities of these substances hereinbefore mentioned, since more may be used if desired, but the benefit derived by larger quantities is rather doubtful.

The proportion of chromium must not be allowed to run much if any above 6% and less than 5% is safer because of a brittle and hot-short condition which is produced. Good results can, however, be obtained down 65 to about 2% of these metals but the air hardening properties are not so pronounced.

The composition or formula above given is that of the furnace charge. The uranium (or equivalent) constitutes primarily a 70 scavenging element and is generally consumed, at least in great part, during the processes of melting, finishing, and casting. The carbon exists as an unwelcome but unavoidable impurity, and care is necessary 75 to maintain the melt as pure as possible. The composition of the finished alloy is preferably substantially the same as that of the charge excepting for the expected disappearance of the uranium as a result of scavenging action. This, as in the case of all metal working, depends largely upon the skill of the melter. One reason why uranium is desirable in this connection is that a slight excess does not injure the resulting alloy as is the case with some scavenging elements. However I have indicated certain equivalents which may be substituted therefor and do not limit myself to the use of uranium.

Little total change is produced in the proportions of chromium, silicon, or iron. Carbon tends to rise but must be kept below 1.00% and preferably below .60%. Accordingly the ultimate composition of the alloy is: Chromium 3% to 6%, silicon 1% to 2½%, uranium and equivalents substantially disappeared, phosphorous, sulphur, manganese as at first, iron to make 100%.

By the term "alloy" I mean any metallic composition of practical value, containing a 100 plurality of metallic ingredients, regardless as to the particular internal structure exhibited thereby.

A casting made from my improved alloy exhibits great toughness, rigidity, strength, 105 and permanence, and possesses an extremely fine and regular crystal formation, together with a tough and silky fracture. This crystal arrangement is not impaired either by prolonged overheating or by sudden chill-

60

65

75

80

85

90

95

100

110

ing. At points above a red heat the alloy can be forged with ease and accuracy and indicates no tendency towards a hot shortness at any temperature. If annealed by 5 long slow cooling, either the casting or forging can be readily machined, and by merely reheating and allowing to cool in the open air will regain such a degree of hardness as is desired for any of the uses above 10 mentioned. This hardness may be regulated by the rate of cooling or may be tempered after sudden cooling (as in oil) by heating to any point short of its temperature of recalescence.

15 This tempering, however, is peculiar in that heating to 1400° Fah. toughens the alloy but does not entirely withdraw its hardness, leaving it hard enough to withstand hot-metal working. Heating does not warp 20 or change the dimensions of a machined article appreciably and produces only an immaterial amount of scale even at 2000° Fah. A machined or finished article can be hardened locally merely by heating very hot at 25 the desired point and allowing to cool.

I have found this alloy a perfect substitute for 10% tungsten steel (which also normally carries 4% of chromium and 1% vanadium) in all uses which have so far come to my attention, and can be made at much smaller 30 cost. This alloy can be made by the electric open hearth, or crucible process and by any of the known processes of making steel.

Having thus described my invention what I claim is:—

1. An alloy consisting essentially of iron containing from about three to about six per cent of chromium and between about one and two and one-half per cent of silicon together with less than one per cent of carbon. 40
2. A furnace charge of the nature described containing essentially: Silicon 1% to 2½%, carbon .30% to 1.00%, chromium 3% to 6%, metallic scavenging element .1% to .3% having the herein essential qualities 45 of uranium, iron to make 100%.

In testimony whereof, I hereunto affix my signature.

HAROLD G. WEIDENTHAL.